

March 3, 1936.

C. P. MARSDEN

2,032,761

FLUORESCENT COATING METHOD

Filed Nov. 21, 1933



Charles P. Marsden  
INVENTOR

BY *John J. Rogan*  
ATTORNEY

## UNITED STATES PATENT OFFICE

2,032,761

## FLUORESCENT COATING METHOD

Charles P. Marsden, Bloomfield, N. J., assignor  
to Hygrade Sylvania Corporation, Salem, Mass.,  
a corporation of Massachusetts

Application November 21, 1933, Serial No. 698,945

5 Claims. (Cl. 91—68)

This invention relates to coating methods and with particularity to coating with fluorescent material.

An object of the invention is to provide a novel 5 method of applying a fluorescent coating to glass or other similar support.

A further object is to provide a novel method of applying a fluorescent coating to a cathode ray tube or similar device.

10 A feature of the invention relates to a cathode ray tube or similar device having a fluorescent coating which has a maximum uniformity.

15 A further feature relates to the method of attaching the fluorescent coating to the glass or other similar body.

Other features and advantages not specifically 20 enumerated will be apparent after a consideration of the following detailed description and appended claims.

25 While the invention finds its greatest practical advantages in the manufacture of so-called cathode ray tubes or Braun tubes, the inventive method is not limited to the manufacture of any particular kind of tube, but is capable of application in any situation where a uniform coating of fluorescent material is to be applied to a supporting member.

In certain types of apparatus, for example 30 cathode ray tubes, Braun tubes, or the like, there is provided a screen which comprises a material that fluoresces or emits light when bombarded by cathode rays or the like. For example, in one known type of construction employed for this purpose, the tube is provided with a constricted 35 or neck portion at one end and an enlarged, substantially flat screen portion at the opposite end, the interior face of this screen portion being provided with this fluorescent coating. Suitable electrodes are provided within the tube for generating, accelerating and oscillating the beam of cathode rays which, upon striking the screen, causes the latter to fluoresce or otherwise emit light rays. Such tubes are customarily used as 40 oscilloscopes for wave analysis, frequency analysis, etc. Tubes of this general type have also been employed for television or picture transmission purposes, in which case the beam or cathode ray not only has its spacial position varied in synchronism with a transmitter, but 45 also the intensity and/or velocity and/or width of the impinging beam are varied to correspondingly vary the intensity of the fluorescent effect from the screen. While, for oscilloscope or similar uses it is important that the fluorescent coating be uniform, minor variations of thickness or

uniformity of the grain in the coating do not seriously affect results. However, in television or similar uses it is absolutely necessary, if truly faithful images are to be reproduced, that the fluorescent coating be not only of the highest 5 uniformity as to thickness, but it is also important that the individual grains constituting the coating be, as far as possible, of the same degree of fineness. It is further highly important in 10 all types of cathode ray tubes that the fluorescent coating be firmly united to the glass or other support, since it is required to be bombarded continuously by the cathode rays.

Various methods have heretofore been proposed 15 for applying the fluorescent coating. For example, the most common way is to mix the fluorescent coating with a suitable binder which is then sprayed over the surface to be coated. Needless to say, with ordinary spraying methods it is extremely difficult to secure a coating of uniform 20 thickness. This may be due to a variety of causes. For example, in spraying it is required that the material be sprayed onto the receiving surface at substantially right angles, with the result that if a non-uniform or large grain of material 25 attaches itself to the supporting surface, succeeding traverses of the spray aggravate and accentuate the thickness of the coating at this point. Added to this is the fact that if the coating is not evenly united to the support over its entire surface, the force of the spray may dislodge one or 30 more grains from the coating. Other methods such as painting or the like obviously are incapable of producing uniform coats because of the 35 appreciable physical dimensions of the painting tool as compared with the fine grain constituting the coating.

It has been found that a thoroughly uniform 40 fluorescent coating may be achieved in accordance with this invention without spray, painting or similar processes.

In accordance with the invention the surface 45 of the tube to be coated is first provided with a tenuous film of tacky or sticky material or a material which exhibits pronounced adhesive properties for the powdered fluorescent material. This fluorescent material is preferably employed in powdered form and preferably mixed with another powdered weighty material such as powdered zinc or the like. The powdered mixture is 50 then poured or deposited in any familiar manner upon the same film to which it adheres. The support is then rotated, oscillated and/or swirled so as to agitate the powdered mixture relative to the said film, thus distributing the fluorescent 55

powdered material in an even deposit over the film. The excess of powdered material may then be removed by pouring or similar process, after which the support may be heated, baked, or fired to a dull red heat to remove the film and/or binders, resulting in a firm attachment of the fluorescent material onto the glass or other support.

While the foregoing description gives a general plan of the preferred procedure to be employed, a detailed description will now be given of the manner of practicing the invention in connection with a typical form of cathode ray tube.

Referring to the drawing, the numeral 1 indicates generally a glass or other tube having a constricted or neck portion 2 and a flared or enlarged portion 3. The portion 3 terminates in a substantially flat portion 4 which serves to carry the fluorescent material. In accordance with well-known practice in the art of cathode ray tube design, the tube 1 is provided with an emitting cathode represented schematically by the numeral 5, and an electrode or electrodes 6 for varying the intensity of the cathode ray beam. A concentrating or focusing electrode 7 is usually provided to restrict the beam to a comparatively narrow width. A pair of vertical deflecting plates 8 and a pair of horizontal deflecting plates 9 (one shown) are provided for oscillating the cathode ray beam over any predetermined path. A suitable anode or anodes 10 are provided for accelerating the electrons from the cathode 5. The manner of producing and oscillating the cathode ray beam above described constitutes no feature of the present invention and any well-known means may be provided for this purpose.

Prior to attaching the constricted or neck portion 2 to the flared portion 1, the latter flared portion 3 has the interior surface of the wall 4 provided with a tenuous film preferably of the nature of a plasticized lacquer indicated in the drawing by the numeral 11. It is preferred to employ a binder consisting of, for example, a solution of nitro cellulose in a volatile solvent, e. g., ethyl carbonate, amyl acetate, etc. This binder solution is then plasticized preferably by mixing with it 1½% dibutyl phthalate, and in order to retard the drying, a small percentage, such as 1% of diethyl oxalate may be mixed with the binder. It is to be understood, of course, that the invention is not limited to this particular plasticizing agent. For example, any diamyl or diethyl phthalate or phthalates may be employed or, if desired, dicesyl phosphate may be employed. The invention also contemplates the use of lacquer films containing gums, if these latter gums are burnt out in the final firing. As above stated, the plasticized film is preferably of a tenuous character or sufficiently thin so as to be substantially completely transparent, although it will be understood that any other known transparent film may be employed which, upon firing, is completely removed or becomes transparent.

The film is preferably deposited by pouring or other similar operation. For example, if the portion 4 of the tube is five inches in diameter, approximately 2 cc. of the above material may be dropped on the interior face of the portion 4 and allowed to flow evenly over the surface. Any excess of the material over the required amount may be drained off in any suitable manner, with the result that there is produced a tenuous uniform film which is substantially free from bubbles, flowing marks, etc. This film is then allowed

to dry or is dried to the point where it becomes appreciably tacky or sticky, and the excess of material around the edges may be wiped off or otherwise removed. The drying is then carried slightly further by blowing a gentle current of air into the bulb until the odor of the solvents has substantially entirely disappeared.

After this treatment the film 11 is in a condition such that it will just show finger prints and is now in condition to receive the powdered fluorescent material. Any well-known fluorescent material such as ordinarily employed in cathode ray tubes or the like may be employed. Preferably this material is intimately mixed with a weighty powdered zinc of about 30 mesh. The mixed powdered materials are then poured into the bulb and the bulb is swirled, oscillated, and somewhat violently shaken so as to distribute the relatively fine fluorescent material in an even deposit over the sticky film 11. As a result of this agitating process the heavy grains or particles of zinc or other weighty material cause the powdered fluorescent material to be distributed in a uniform layer over the film 11. One possible explanation for this is that the very fine particles of the fluorescent material are held by a sufficient adhesive force to prevent their dislodgment by the moving or swirling weighty particles of zinc, whereas the non-uniform or enlarged grains of the fluorescent material are carried by the swirling or agitated weighty material, with the result that the fluorescent coat which finally adheres to the film 11 consists of substantially uniform and finely grained fluorescent material. The excess of the powdered materials may then be poured out or otherwise removed from the tube. If, upon examination of the tube, it is discovered that there is an excess of fluorescent material forming a lump at any particular portion of the film, this can be removed by adding more zinc or similar weighty material and continuing the swirling action until the lump or non-uniformity is removed. The material having thus been removed, the edges of the coating may be trimmed by rotating the bulb and wiping off the material with a cloth or rubber scraper.

The end 4 of the tube is then subjected to heat, preferably to raise it to a dull red heat or to a temperature at which the binder and/or the plasticized film 11 is removed. Preferably also, the heat is maintained for a sufficient length of time to take the fluorescent material onto the member 4.

A tube prepared in accordance with the above coating has been found to possess extremely uniform graining and thickness of fluorescent material and it will be obvious, of course, that various changes and modifications may be made in the described procedure without departing from the spirit and scope of the invention. For example, if desired the portion 4 of the tube may be slightly heated while pouring in the plasticized lacquer, and this heating may be gradually increased until the film is entirely removed.

If desired, the above procedure may be repeated so as to provide successive coats of fluorescent material, each coating having a thickness practically consisting of a single grain.

The portion 3 thus prepared may then be united or sealed to the neck portion 2 and the tube may then be subjected to the ordinary evacuation and treatment customarily employed in the manufacture of vacuum tube and electron tube devices in general.

It has been found that the foregoing method

renders it possible to vary the thickness of the fluorescent coating from an almost transparent one to an almost opaque one—

5 (1) By varying the tackiness of the binder coating either by varying the quantity of plasticizer that is used, or by regulating the extent of drying of the film before applying the powdered material;

10 (2) By varying the magnitude or velocity of the swirling action given to the powdered material.

This application is a continuation-in-part of application Serial No. 674,047, filed June 2, 1933.

What I claim is:

15 1. The method of applying a coating of powdery fluorescent material containing fine and coarse grains to a cathode ray tube which comprises, flowing onto said support a smooth thin film of a plasticized lacquer binder solution, drying said film until the odor of the solvents is substantially entirely removed and said film becomes appreciably tacky, depositing said powdery material on said film, and swirling said support to cause the coarser grains of said material to distribute the finer grains of said material in a uniform layer on said film, removing any excess of said material, and heating the support to remove excess lacquer and to bake said powdery material on said support.

20 2. The method of providing a cathode ray tube with a uniform coating of powdery fluorescent material which comprises, flowing onto a wall of said tube a thin film of a plasticized binder solution, drying said solution to the point where it becomes appreciably tacky and the odor of the solvents is substantially entirely removed, mixing with the powdery fluorescent material

another powdery material of greater weight than the fluorescent material, depositing said mixture on said film, swirling and shaking said tube to distribute said fluorescent material in a substantially uniform layer, removing any excess of said mixture, and heating the wall of said tube to bake said powdery material thereon.

25 3. The method of applying a uniform coating of fluorescent material to a cathode ray tube which comprises, flowing onto a wall of said tube a thin film of a transparent plasticized lacquer, mixing with the powdery fluorescent material a quantity of powdery material which is heavier than the powdery fluorescent material, depositing said mixture on said film while said film is appreciably sticky, swirling and shaking said mixture until lighter grains are distributed in a uniform layer over said film, removing excess of said mixture, and heating the wall of the tube to bake the powdery material thereon.

30 4. The method of providing a cathode ray tube with a fluorescent coating which comprises, mixing a phthalate with a nitrocellulose binder, depositing said mixture in a thin film onto a wall of said tube, drying said film until the solvents are substantially entirely removed, mixing with the fluorescent material another weightier powdered material, swirling the tube to cause the weightier material to distribute the grains of the fluorescent material uniformly over said film, and subsequently heating said film to remove said binder.

35 5. The method according to claim 4 in which the fluorescent material is mixed with a powdered zinc of approximately 30 mesh.

CHARLES P. MARDEN.